

# UNITED STATES PATENT OFFICE.

LUCIUS D. CHAPIN, OF CHICAGO, ILLINOIS.

## MANUFACTURE OF WROUGHT-IRON.

SPECIFICATION forming part of Letters Patent No. 283,074, dated August 14, 1883.

Application filed October 3, 1881. (No specimens.)

*To all whom it may concern:*

Be it known that I, LUCIUS D. CHAPIN, a citizen of the United States, residing at Chicago, in the county of Cook and State of Illinois, have invented certain new and useful Improvements in the Manufacture of Wrought-Iron; and I do hereby declare the following to be a full, clear, and exact description, sufficient to enable others skilled in the art to which said invention appertains to make and use the same.

In the manufacture of wrought-iron as ordinarily practiced the charge of cast-iron is subjected to the reducing action of the furnace-gases on a reverberatory hearth having a "fix" or "fettle" made up in considerable measure of iron oxide, either in the form of ore or of mill-cinder, scale, or the like. The presence of the oxide lining is deemed highly essential to the successful working of the charge, for without it when the metal comes to "nature" and is in pasty condition ready to be collected into a ball or loop, the wrought-iron adheres tenaciously to the silicious lining, thus making it extremely difficult to work into a mass, and then only at a great loss of the metal. Hence it is that to avoid the difficulty precaution is taken to supplement the usual lining with charges of iron oxide in various forms and combinations spread upon the hearth above the same and next in contact with the molten metal. Practice has demonstrated that in this way the cast metal may be reduced to wrought-iron with entire economy, save that after each heat, or at best after very few heats, it is necessary to renew the iron-oxide lining, which not only consumes time in bringing the furnace again into "condition," but is wasteful, moreover, of crude materials rich in iron. The present invention has for its object to avoid this repeated and necessarily expensive renewal of the oxide lining in manufacture of wrought-iron, and is based upon the discovery that, if the crude cast-iron be subjected to a preliminary treatment in a pneumatic converter having the usual lining of fire-brick, ganister, or like silicious material until said cast-iron is practically free from silicon and a large per centum of its carbon, the iron may

having an iron-oxide lining, and therein speedily reduced to a wrought condition without material loss of oxide lining, and consequently without the frequent renewal of said lining which the methods of manufacture heretofore in vogue have made necessary. 55

In Letters Patent granted to me January 13, 1880, No. 223,481, I have described and claimed a process or method of making wrought-iron wherein the molten metal, while 60 inclosed in a converter, was subjected simultaneously to the oscillatory or rotary action of the converter and to the action of an air-blast until it approaches nature, with an occasional intermitting or varying of one action or the other, as therein described, if so required, after which the metal was transferred to a separate furnace or balling-chamber and balled under a reverberatory heat or flame. The form of converter shown in said patent and 65 described as preferable is somewhat of the type or kind commonly known as the "Danks furnace," and with such a converter I contemplated the use of a lining somewhat like the one commonly used in the Danks furnace, 70 and which in its characteristic features resembles the lining, fix, or fettling usually employed in puddling or boiling furnaces. Such linings have usually a considerable percentage of oxide of iron or other metallic elements, 75 which are supposed to "nourish" the iron under treatment and to facilitate its coming to nature. It was with reference to the use of linings of that general class that I described the oscillatory or rotary motion of the converter more or less intermittently as an element of the invention set forth in said patent. If, instead of said non-refractory linings having 80 a considerable percentage of iron oxide or other metallic elements in their composition, the lining of the converter be of fire-brick, ganister, or like silicious material, I have found, first, that it is unnecessary to impart to the converter any oscillatory or rotary motion during the first stage of the process; second, that in subjecting the molten metal to the action of the air-blast alone for a few minutes until it more or less approaches nature or comes to a degree of conversion corresponding thereto, the 85 refractory lining is attacked but slightly, and, 90 95 100

indeed, very much less than when a non-refractory lining is employed, as specified, thus saving the expense of frequent renewal; while, third, the iron is left in such purified condition that, upon subsequent transfer to a baller having a metallic lining usual to a puddling, balling, or Danks furnace, it can be speedily reduced therein to a wrought condition under influence of a reverberatory flame with practically little or none of the disastrous "cutting" of the lining which has been heretofore experienced.

In the practice of my present invention I use for a converter a horizontal cylindrical chamber—such as is called for in said Patent No. 223,481—having an air-blast or an ordinary Bessemer converter, or any other desired form of chamber suitable for the purpose, but having an air-blast such, or substantially such, as the Bessemer operation calls for. Such converter may be mounted upon trunnions for convenience in charging and removing the charge, or it may be fixed in position and provided with a charging-hole and tap-hole, as such devices are known in the art. The converter is to be lined with ganister or fire-clay or other suitable refractory material, and especially excluding any such percentage of metallic oxide as is usually employed in the Danks or in ordinary puddling or boiling furnaces.

The charge of metal may be run in from a cupola or blast furnace, and then treated with the air-blast substantially as described in said Patent No. 223,481, except that the converter need not be rotated or oscillated during the blowing of the blast, nor need the metal have any other motion imparted to it than what results from the blowing of the blast. The blast is kept blowing for a short time—say, for ten minutes, more or less—either till the metal approaches nature or comes to or approaches a corresponding degree or stage of purification, or it may be arrested somewhat sooner, though in the latter case the subsequent operations in the baller or balling-furnace will require more time; but in any case the metal should be kept under the air-blast treatment in the converter until the objectionable impurities which the air-blast is adapted to remove shall have been substantially eliminated, or so far eliminated that the presence of the residue will not in subsequent working prevent the production of good iron. The metal is next tapped, run or otherwise transferred to a baller or balling-chamber having any lining such as is adapted to nourish the iron or aid in fluxing or decarbonizing or otherwise completing its conversion and bringing it completely to nature, and such baller or balling-chamber may be of any construction and operation, provided, only, it be of such as to admit of the use of a reverberatory heat or flame on the iron under treatment therein, and also permit the use of motion imparted mechanically to the iron, preferably by the rotary or oscillatory motion of the baller or balling-chamber itself. The me-

chanical work of balling the iron under such conditions and of removing the ball and further working it is so well known in the art that further description is unnecessary.

In practice of the process as above described I have found that the quality of the iron is materially improved; that the labor and expense of its production is much lessened by doing away with the constant repairs to the converter-lining made necessary when this was of non-refractory materials, and that by the subsequent transfer of the metal to the baller after the first part of the process of conversion carried on in the converter has been finished the lining of the baller is slightly, if at all, impaired, or, if impaired, is replenished as much, or nearly as much, as it is worn away, and thus becomes practically self-sustaining. This is a great economy as compared with any process with which I am familiar. The whole expense, or nearly so, of "fix" or "fettling" is avoided in the baller when once lined, while the refractory lining of the converter is very permanent as compared with the lining of an ordinary puddling or boiling or Danks furnace.

By the foregoing treatment the molten charge of iron as it leaves the converter is so far advanced to a wrought condition that only a few minutes' exposure in the balling-chamber is necessary to perfect the reduction and allow for the formation of the loop. It is plain that the process as defined is very expeditious in comparison with the older methods of making wrought-iron, and has, besides, the merit of working upon large masses of metal, insuring greater homogeneity for a larger product.

Prior to the invention it has been proposed to partially decarburize and desiliconize a charge of molten cast-iron by an oxidizing-blast in a pneumatic converter, and thereafter to transfer the metal to an open hearth having a refractory lining of sand, fire-clay, ganister, or the like, wherein it is subjected to a reverberatory flame and to the actions of titaniferous-iron oxide and basic fluoride additions in conjunction; but these materials are designed to free the iron of its phosphorus and sulphur, requires several hours to perfect their action, the metal is in molten condition throughout, and is finally cast in ingots and not reduced to a puddled ball, as herein defined. The product thus obtained is somewhat malleable, but is in no sense wrought-iron, nor does its course of treatment give any clue to the conditions under which wrought-iron may be produced.

Having thus described the invention, what I claim as new, and desire to secure by Letters Patent, is—

1. The process of making wrought-iron which consists in subjecting molten cast-iron, in a Bessemer converter having a fire-brick, ganister, or like silicious lining to the action of an air-blast until the objectionable impurities, which the air-blast is adapted to remove, shall have been substantially eliminated, and then transferring the metal to a separate fur-

nace or balling-chamber having essentially an oxide-of-iron lining, and therein subjecting it to reverberatory flame and to puddling action until it is reduced to a wrought condition to 5 form a ball or loop, substantially as described.

2. The process of making wrought-iron which consists in subjecting molten cast-iron, in a Bessemer converter having a refractory lining to the action of an air-blast until the 10 objectionable impurities, which the air-blast is adapted to remove, shall have been substantially eliminated, and then transferring the

metal to a separate furnace or chamber, and therein subjecting it to a reverberatory flame and to a rotary puddling action until it is reduced to a wrought condition to form a ball or loop, substantially as described. 15

In testimony whereof I have hereunto set my hand.

LUCIUS D. CHAPIN.

Witnesses:

M. T. HUGGINS,  
M. F. CHAPIN.